

# United States Patent

Van Allan et al.

[15] 3,642,479

[45] Feb. 15, 1972

[54] **PHOTOGRAPHIC ELEMENT AND PROCESS**

[72] Inventors: James A. Van Allan; Dennis E. De Meyer, both of Rochester, N.Y.; Frank D. Allen, deceased, late of Rochester, N.Y.

[73] Assignee: Eastman Kodak Company, Rochester, N.Y.

[22] Filed: Mar. 2, 1970

[21] Appl. No.: 15,867

[52] U.S. Cl.....96/48 R, 96/90, 96/90 PC

[51] Int. Cl.....G03c 5/24, G03c 1/72

[58] Field of Search.....96/90, 90 PC, 48

3,121,633 2/1964 Sprague et al. ....96/90  
3,532,638 10/1970 Otis.....96/90 PC X

Primary Examiner—Norman G. Torchin

Assistant Examiner—Richard E. Fichter

Attorney—W. H. J. Kline, J. R. Frederick and D. M. De Leo

[57] **ABSTRACT**

Photographic elements having a support on which is coated a layer including a light-sensitive halocarbon and a 1,4-pyran derivative like 1-(p-N,N-dimethylaminophenyl)-1H-3-(p-ethoxyphenyl)naphtho[2,1-b]pyran or 4-(p-N,N-dimethylaminophenyl)-2-phenyl-4H-1-benzof[b]pyran yield printout images in exposed areas on exposure to actinic rays. The resultant printout image can be intensified by heating.

[56] **References Cited**

UNITED STATES PATENTS

3,486,899 12/1969 Brown .....96/90

**9 Claims, No Drawings**

## PHOTOGRAPHIC ELEMENT AND PROCESS

This invention relates to photography and particularly to photographic elements and processes for forming printout images.

It is known that certain halocarbons and polyhalocarbons are light sensitive and yield photographic products which are capable of producing colored materials from such colorless materials as certain dyes, and diarylamines. Examples of this light sensitivity can be found in Mechanisms and Structures In Organic Reaction, Gould, page 744; and in U.S. Pat. Nos. 3,102,810 and 3,121,633; in British Pat. Nos. 916,779 and 719,919. These references are based on the photoreaction of polyhalocarbons with leuco dyes to yield the corresponding colored forms of the dyes.

While polyhalocarbons having been employed separately as light-sensitive addenda for certain photographic processes and elements. They have not been combined with 4H-pyran derivatives to prepare photographic printout elements.

Accordingly, an object of this invention is to provide novel photographic elements.

Another object of this invention is to provide new photographic elements useful in preparing printout images.

Still another object of the present invention is to provide novel photographic elements including, as the image-forming components, at least one halocarbon and at least one 4H-pyran derivative.

An additional object of this invention is to provide a new photographic process for producing printout images.

Other objects and advantages of this invention will become increasingly apparent from a reading of the following specification and appended claims.

The objects of this invention are accomplished both with photographic elements wherein a support is coated with a layer including a light-sensitive halocarbon and a 4H-pyran derivative and with a photographic process for the preparation of printout images including imagewise exposing an element such as described above to actinic rays.

4H-pyran derivatives useful in the photographic elements of this invention include those having at least one aromatic substituent on the pyran ring. Especially desirable are those substituted at the 2-position and at the 4-position, with at least one of these substituents being an aromatic radical which itself can be still additionally substituted. Additionally the pyran nucleus is desirably fused to an aromatic nucleus to form, for example, a benzopyran or a [2,1-b]naphthopyran.

Particularly advantageous pyran derivatives include those having the formula:



wherein

- each of R and R<sup>1</sup> represent either a hydrogen atom, an alkyl radical or an aryl radical and at least one of R or R<sup>1</sup> is an aryl radical,
- each of R<sup>2</sup> and R<sup>3</sup>, when taken alone, represents a hydrogen atom, and
- R<sup>2</sup> and R<sup>3</sup>, when taken together, represent the atoms necessary to complete an aromatic ring system.

As defined herein, the term alkyl radical refers to straight and branched chain alkyl radicals having from one to about four carbon atoms like methyl, ethyl, 2-methoxyethyl, propyl, isopropyl, n-butyl, or the like, etc. The alkyl radical can be additionally substituted, e.g., ethoxycarbonylcyanomethyl, ethoxycarbonylbenzoylmethyl, nitromethyl, etc. Alkoxy radical refers to alkoxy radicals having from one to about four carbon atoms such as methoxy, ethoxy, propoxy, butoxy, etc., and preferably methoxy or ethoxy. The term aryl radical designates aromatic substituted or unsubstituted aryl radicals

having from six to 10 carbon atoms in the nucleus, and including such aryl radicals as phenyl, naphthyl, p-tolyl, p-ethoxyphenyl, p-dimethylaminophenyl and the like. Also as used herein, the designation aromatic ring system refers to a mono or poly cyclic, carbocyclic aromatic nucleus like benzene, naphthalene, anthracene, phenanthrene, etc., which is completed by the atoms represented by R<sup>2</sup> and R<sup>3</sup> taken together and is fused to the parent pyran ring between the adjacent carbon atoms substituted by R<sup>2</sup> and R<sup>3</sup>.

Especially advantageous pyran derivatives as described herein include those wherein R represents either a hydrogen atom, a methyl radical, an N,N-dimethylaminophenyl radical or a p-methylphenylthio radical and R<sup>1</sup> represents a phenyl radical including substituted phenyl radicals like p-ethoxyphenyl, N,N-dimethylaminophenyl and the like. Still other especially desirable pyran compounds include those wherein R<sup>2</sup> and R<sup>3</sup>, when taken together, represent a 1,4-buta-1,3-dienylene radical (i.e., —CH=CH—CH=CH—) with R<sup>2</sup> and R<sup>3</sup> thereby completing a benzene nucleus.

Preferred 4H-pyran derivatives useful in the photographic elements of this invention include

TABLE I

| Compound No. |
|--------------|
| 1            |
| 2            |
| 3            |
| 4            |
| 5            |
| 6            |
| 7            |
| 8            |
| 9            |
| 10           |
| 11           |
| 12           |

1-(p,N,N-dimethylaminophenyl)-1H-3-(p-ethoxyphenyl)naphtho[2,1-b]pyran,  
 1-(p,N,N-dimethylaminophenyl)-1H-3-phenylnaphtho[2,1-b]pyran,  
 4-(p,N,N-dimethylaminophenyl)-2-phenyl-4H-1-benz[1-b]pyran,  
 2-(p,N,N-dimethylaminophenyl)-4H-benz[1-b]pyran  
 1H-3-(p,N,N-dimethylaminophenyl)naphtho[2,1-b]pyran,  
 2-phenyl-4H-benz[1-b]pyran,  
 1-(p-tolylthio)-1H-3-(p-ethoxyphenyl)naphtho[2,1-b]pyran,  
 2-ethoxyphenyl-4-(p-tolylthio)-4H-benz[1-b]pyran,  
 1-(1-ethoxycarbonyl-1-cyanomethyl)-1H-3-(p-ethoxyphenyl)naphtho[2,1-b]pyran,  
 4-(1-ethoxycarbonyl-1-cyanomethyl)-2-phenyl-4H-benz[1-b]pyran,  
 1-(1-ethoxycarbonyl-1-benzoylmethyl)-1H-3-(p-ethoxyphenyl)naphtho[2,1-b]pyran, and  
 1-nitromethyl-1H-3-(p,N,N-dimethylaminophenyl)naphtho[1-b]pyran.

Also included in the present photographic elements, in combination with at least one pyran derivative like those mentioned hereinabove is at least one halocarbon or polyhalocarbon compound. The pyran derivatives and halocarbon compounds are generally combined herein in weight ratios of from about 3:1 to about 1:5 respectively, and preferably in substantially equal amounts by weight. Useful halocarbon compounds include, for example,  $\alpha$ -halocarbonyl compounds like  $\alpha,\alpha,\alpha$ -tribromoaceto-phenone, poly(vinyl halides) such as poly(vinyl bromide) as well as perhalides and the like. Especially desirable halocarbon compounds are those known to be decomposed by exposure to actinic rays (i.e., ultraviolet and blue light) and which are not acidic. Preferred halocarbon compounds of this type include polyhalocarbons having three halogen atoms chemically bonded to a terminal carbon atom, i.e., those having the formula  $R^2-C-(X)_3$  wherein X represents a halogen atom and R<sup>2</sup> represents either a halogen atom, an alkyl radical, a haloalkyl radical, an aryl radical or an aryl radical. Exemplary polyhalogens include such compounds as polyhaloalkanes like iodoform, carbon tetrabromide, pentabromoethane, hexabromoethane, hexachloroethane and tribromophenylmethane. Bromo and iodo compounds are especially preferred due to their inherently greater light sensitivity as compared to that of the corresponding chloro compounds. Polyhalocarbons, such as iodoform,

which can be inactivated or diffused from a coated layer on heat treatment are also preferred since they permit convenient stabilization of the photographic image by the application of heat.

In addition to pyran derivatives and halocarbon compounds, the photographic elements of this invention can contain additional addenda, e.g., sensitizers or addenda to enhance storage stability or either image quality or raw stock or image stability. As an example, certain nitrogen containing compounds promote the photographic speed and resultant image density at any given exposure level. These materials are well known in the photographic art and include such compounds as 5-dimethylaminocoumarin, 6-diethylamino-4-methylcoumarin, carbazole, diphenylformamide, 4-dimethylaminobenzaldehyde, phenothiazine and the like.

As well as sensitizing addenda, materials which inhibit premature reaction in the sensitive layers are useful inclusions. Presumably, such compounds, which can be included singly or in combination and admixture, function to buffer the image-forming components against a pH change, i.e., to an acidic pH, which would promote a premature printout reaction. Desirable stabilizing materials include nitrogen-containing heterocycles like benzimidazole, 2-methylbenzimidazole, 2-styrylbenzimidazole as well as related nitrogen containing compounds such as azoles like isoazole, triazole, benzotriazole, etc.; azine compounds like pyrimidine, pyrazine, benzopyrimidine and other diazines or triazine compounds such as 1,2,4-triazine, 1,2,3-triazine, 1,3,5-triazine, etc.

Other useful addenda materials include image stabilizers, they being compounds which enhance the resistance of a resultant photographic image against deterioration from subsequent exposure to heat, light or the like energies which can cause fading or discoloration of the image. Exemplary such stabilizers include thiazine compounds like phenothiazine and oxines such as alkoxyboroxines.

Generally, the image-forming components and additional stabilizing or other modifying addenda are dispersed in a hydrophobic film-forming resin binder to promote the formation of a coated layer. Desirable resinous matrix vehicles include those which have a softening point sufficiently high to resist tackiness at the temperature ranges, i.e., up to about 150° C., useful for intensifying or stabilizing photographic images produced on elements of this invention. Additionally, the pH of the resin binder should not be such that it either promotes or unduly inhibits, i.e., more than do the described stabilizers, the image-forming reaction. Exemplary matrix vehicles, having the noted characteristics, can be selected from a wide variety of materials, including natural resins, modified natural resins and synthetic resins. Exemplary useful natural resins are balsam resins, colophony and shellac. Exemplary suitable modified natural resins are colophony-modified phenol resins and other resins listed below with a large proportion of colophony. Suitable synthetic resins include the extensive variety of synthetic resins, for example, polymers, such as vinyl polymers including a polyvinyl chloride, polyvinylidene chloride, polyvinyl acetate, polyvinyl acetals, polyvinyl ether and polyacrylic and polymethacrylic esters; polystyrene and substituted polystyrenes or polycondensates, e.g., polyesters, such as phthalate resin, terephthalic and isophthalic polyesters, maleinate resin and colophony-mixed esters of higher alcohols; phenol-formaldehyde resins, including colophony-modified phenol-formaldehyde condensates, aldehyde resins, ketone resins, polyamides and polyadducts, e.g., polyurethanes. Moreover, high-melting polyolefins, such as various polyethylenes, polypropylenes, polyisobutylenes and chlorinated rubber are suitable. Additional useful resinous binder materials are known to those skilled in the polymer arts.

To prepare a composite photographic element of this invention, the image-forming components and such supplemental addenda compounds as are desired are generally dissolved or dispersed in a solution of matrix vehicle to prepare a coating

composition which can then be applied to a support material by solvent coating techniques. In a coating formulation, the halocarbon and pyran derivative are generally present in stoichiometric amounts or with an excess of pyran derivative. 5 Modifying addenda, if included, can be present in widely varying amounts and the chosen amount will depend on both the selection and quantities of image-forming components as well as the modifying effect desired. Conventionally they are included in an amount of from about 1 to about 35 percent by 10 weight of the image-forming ingredients. The image-forming compositions, including stabilizers or other modifying addenda are generally incorporated into a coating formulation in an amount of from about 5 to about 50 parts by weight per 15 100 parts by weight of matrix vehicle. Advantageously, the composite coating formulation contains from about 5 to about 20 weight percent solid for ease of coating, although wider variations can be used if desired for particular situations.

Coating can be accomplished by a wide variety of 20 techniques including flow coating, doctor blade coating, whirl coating, extrusion hopper coating, etc. The support material onto which the light-sensitive layer is applied is widely variable and includes such supports as cellulosic materials like cellulose acetate, cellulose acetate butyrate, etc., as well as polystyrenes, polycarbonates, polyvinyl compounds like polyvinylacetals, polyesters such as poly(ethylene terephthalate), poly- $\alpha$ -olefins like polyethylene, polypropylene and other poly- $\alpha$ -olefins conventionally having from two to 10 carbon atoms, and including metals like zinc and aluminum and paper including polyethylene and polypropylene coated papers.

Subsequent to coating and drying to form a composite photographic element of this invention, the resultant element 35 can be imagewise exposed to actinic rays to prepare visible printout images. After exposure, heating like that previously described can be employed to intensity or stabilize the light-induced photographic image. Stabilization, as noted above, is accomplished by exhausting unreacted halocarbon from the 40 layer. Intensification results from the heat promoted action of an image intensifier like those described herein. Desirably, heating is within a range of from about 100° to about 150° C., but wider variations in temperature can be used if desired.

The following examples are included for a further understanding of the invention.

#### EXAMPLE 1

A solution of 0.15 g. of compound 1, from Table I, 0.15 g. of 50 6-diethylamino-4-methylcoumarin, 0.3 g. of carbon tetrabromide, and 0.03 g. of 2-methylbenzimidazole in 4 ml. of dichloroethane is added to 11 ml. of a 10 percent solution of poly(vinyl butyral) dichloroethane and methanol (5:1). The resulting solution is doctor blade coated on a paper support at 55 a wet thickness of 0.004 inch and allowed to dry. The resultant element is then exposed through a negative transparency in an Ozamatic Printer, manufactured by the Ozalid Corp., at a linear transport speed of 8 ft./min. to obtain a dark green, positive image on a white background. The Ozamatic printer uses a 1,200 watt high-pressure mercury arc lamp as an exposure source. Heat treatment for 10 seconds at 150° C. increases the image density, and stabilizes the print against further light reaction.

#### EXAMPLE 2

A solution of 0.15 g. of compound 3, from Table I, 0.15 g. of 6-diethylamino-4-methylcoumarin, 0.35 g. of carbon tetrabromide, and 0.03 g. of 2-methylbenzimidazole in 4 ml. of dichloroethane is added to 11 ml. of a poly(vinyl butyral) solution as in Example 1. The resulting solution is doctor blade coated on a paper support at a wet thickness of 0.004 inch and allowed to dry. The resultant element is then exposed and heated as in Example 1 to obtain an intensified, stable 70 dark blue image on a light blue background.

## EXAMPLE 3

To 4 ml. of a 10 percent solution of a styrene-butyl-methacrylate copolymer in dichloroethane is added a solution of 25 mg. of compound 1 from Table I, 25 mg. of carbon tetrabromide, 2.5 mg. of 2-methyl-benzimidazole, and 10 mg. of 6-diethylamino-4-methylcoumarin in 1 ml. dichloroethane. This solution is doctor blade coated on a paper support at a wet thickness of 0.004 inch and allowed to dry. The resultant element is exposed as in Example 1, but at a linear speed of 5 ft./min. Heat treatment at 150° C. for 10 seconds gives an intensified dark green, positive image on a white background.

ratio of from 3:1 to 1:5 respectively.

2. A photographic element as described in claim 1 wherein the halocarbon compound is selected from the group consisting of halocarbon and polyhalocarbon compounds and wherein the 4H-pyran derivative has the formula:



wherein

a. each of R and R<sup>1</sup> represent a member selected from the group consisting of a hydrogen atom, an alkyl radical and an aryl radical and at least one of R and R<sup>1</sup> is an aryl radical,

b. each of R<sup>2</sup> and R<sup>3</sup>, when taken alone, represents a hydrogen atom, and

c. R<sup>2</sup> and R<sup>3</sup>, when taken together, represent the atoms necessary to complete an aromatic ring system.

3. A photographic element as described in claim 2 wherein R represents a radical selected from the group consisting of a hydrogen atom, a methyl radical, an N,N-dimethylaminophenyl radical, and a p-methylphenylthio radical and R<sup>1</sup> represents a phenyl radical.

4. A photographic element as described in claim 2 wherein R<sup>2</sup> and R<sup>3</sup>, when taken together, represent a 1,4-but-1,3-dienylene radical.

5. A photographic element as described in claim 3 wherein the methyl radical represented by R is selected from the group consisting of a 1-ethoxycarbonyl-1-cyanomethyl radical, a 1-ethoxycarbonyl-1-benzoylmethyl radical and a nitromethyl radical and the phenyl radical represented by R<sup>1</sup> is selected from the group consisting of a phenyl radical, a p-ethoxyphenyl radical and a p-dimethylaminophenyl radical.

6. A photographic element for the production of printout images and comprising a support having coated thereon a layer comprising a halocarbon selected from the group consisting of carbon tetrabromide and dichloroethane and a 4H-pyran derivative as described in claim 3.

7. A photographic element for the production of printout images and comprising a support having coated thereon a layer comprising a carbon tetrabromide and a 4H-pyran derivative selected from the group consisting

a. 1-(p-N,N-dimethylaminophenyl)1H-3-(p-ethoxyphenyl)naphtho[2,1-b]pyran

b. 4-(p-N,N-dimethylaminophenyl)-2-phenyl-4H-1-benzo[b]pyran

c. 1H-3-(p-N,N-dimethylaminophenyl)naphtho[2,1-b]-pyran

d. 1-(p-tolylthio)-1H-3-(p-ethoxyphenyl)naphtho-[2,1-b]pyran

e. 1-(1-ethoxycarbonyl-1-cyanomethyl)-1H-3-(p-ethoxyphenyl)naphtho[2,1-b]pyran

f. 4-(1-ethoxycarbonyl-1-cyanomethyl)-2-phenyl-4H-benzo[b]pyran

g. 1-(1-ethoxycarbonyl-1-benzoylmethyl)-1H-3-(p-ethoxyphenyl)naphtho[2,1-b]pyran

h. 1-nitromethyl-1H-3-(p-(N,N-dimethylamino)phenyl)-naphtho[2,1-b]pyran,

said pyran and said carbon tetrabromide being combined in a weight ratio of from 3:1 to 1:5 respectively.

8. A photographic image-forming process for the preparation of printout images on a photographic element as described in claim 1, which process comprises imagewise exposing said element to actinic rays, whereupon a printout image is produced in exposed areas.

9. A photographic image-forming process as described in claim 8 and additionally including heating said exposed element to intensify the printout image.

\* \* \* \* \*